# EUROPEAN PATENT SPECIFICATION

(11) **EP 0 223 355 B1**
(45) Date of publication and mention of the grant of the patent: **11.10.1989**
(21) Application number: 86307049.6
(22) Date of filing: 12.09.1986
(51) Int. Cl.: H01B 1/24

(54) **Method of manufacturing a pressure-sensitive conductive elastomer compound**
Verfahren zur Erzeugung eines druckempfindlichen leitfähigen Verbundelastomers
Procédé de fabrication d'un composé élastomère conducteur sensible à la pression

(30) Priority: 11.11.1985 JP 253525/85
(43) Date of publication of application: 27.05.1987
(73) Proprietor: NITTA INDUSTRIES CORPORATION, Chuo-ku Osaka (JP)
(72) Inventor: Takaya, Mitsuo, Nara-shi Nara (JP); Inoue, Kiyotaka, Yamatokooriyama-shi Nara (JP); Higuchi, Katsumi, Yamatokooriyama-shi Nara (JP)
(74) Representative: Barker, Rosemary Anne

(56) References cited:
- FR-A- 2 450 856
- FR-A- 2 537 984

## Description

This invention relates to a method of manufacturing a pressure-sensitive conductive elastomer compound of the type exhibits high resistance (insulating performance) when it is in non-pressed condition, and of which the resistance, as the compound is pressed, will vary according to the magnitude of the pressure.

Hitherto, pressure-sensitive conductive materials have been known which are in the form of a compound comprising a resilient material, such as rubber or the like, and a conductive filler mixed therewith. In this respect, metallic particles, such as nickel, conductive carbon black, graphite particles and the like are normally used as the filler. Such conductive compounds, moulded into rod or sheet form, are widely used today as switching elements, are as pressure-sensitive elements for sensors such as pressure sensors and tactile sensors.

A number of problems are associated with conductive compounds of the aforesaid conventional type. Those incorporating metallic particles as a conductive filler are liable to a change of properties with time due to oxidation of the particles. Thus, such compounds lack stability and are often subject of chattering and noise generation. Those incorporating powdery masses of conductive carbon black as a conductive filler exhibit insignificant change in resistance when they are under pressure, because the particle diameter of the carbon black is extremely small, i.e. only 20 to 30 mp. As such, these latter compounds are of no practical use. Finally, if a granulated material formed of conductive carbon black is used as a filler, it is possible to obtain greater variations in resistance, but a conductive compound incorporating such material is liable to particle breakage when it is under pressure. Thus, such compound lacks both durability and stability.

If graphite particles are used as a conductive filler, no characteristic stability can be obtained if they are of non-uniform shape, as in natural graphite. Therefore, it is known to use artificial graphite particles which have been rounded and freed of sharpness by pulverization, or milling, or otherwise, to provide good characteristic stability. Conductive compounds incorporating artificial graphite particles of such type are advantageous in that they are characteristically stable, durable, and less liable to noise generation than other types of compound. On the other hand they have drawbacks in that preparation of graphite particles to the desired configuration requires a complicated and troublesome procedure and in that the attainable yield thereof is rather low.

In view of the aforesaid difficulties with the prior-art compounds, this invention has as its primary object the provision of a pressure-sensitive conductive elastomer compound which has high stable conductive characteristics under pressure and which is also easy to manufacture.

Another object of the invention is to provide a pressure-sensitive conductive elastomer compound whose conductive characteristics under pressure may be varied without changing the mechanical properties of the compound.

In order to accomplish the above and other objects according to the invention a method of manufacturing a pressure-sensitive conductive elastomer compound comprises the steps of:
(a) forming spherical particles of macromolecular material of 30 to 120 um in diameter by chemical pulverization or suspension polymerization;
(b) at least partially carbonizing said spherical particles by baking them within inert gas (without addition of carbon); and
(c) incorporating and dispersing the resultant carbonized spherical particles into a matrix material having insulating and elastomeric properties, the proportion of particles to the entire compound being 20 to 60% by volume.

Materials which may by used as the aforesaid matrix material having insulating and elastomeric properties include natural rubber; synthetic rubbers, such a chloroprene rubber, SBR, NBR, and silicone polyester, and EVA: and liquid rubbers, such as polyurethane and silicone. Particularly preferable among them is a silicone rubber, material having a high heat resistance, excellent electrical properties, and good resistance to chemicals.

Macromolecular materials having a spherical particle configuration useful for the purpose of the invention include styrene, vinylchloride, vinylidene-chloride, methyl methacrylate, and furfuryl alcohol, all prepared in spherical particle form by suspension polymerization, and resol resins chemically pulverized into spherical partical form.

The term "suspension polymerization" referred to herein means a process where a polymerization catalyst is added to monomers, the mixture being stirred in water with a dispersant added to allow the monomers to disperse in oil-drop form and then polymerize.

The term "chemically pulverized" referred to herein means a process whereby a resin dissolved in a solvent is cooled or added to a precipitant so that the resin is separated out in fine powder form.

The particle diameter of the conductive particles in the compound of the invention is from 30 to 120 pm, preferably from 50 to 100 um, and the proportion of the particles to the compound as a whole is 20% to 60% by volume. If the particle diameter is less than 30 itm, the possible variation in resistance of the compound is extremely small, while if it is greater than 120um, the particles cannot satisfactorily be dispersed in the matrix material. The proportion by volume of the particles may be suitably determined according to the desired characteristics and sensitivity of the compound, and also taking into account the type of matrix material. However, if it is less than 20% by volume, the compound may not exhibit sufficient conductivity, and if it is more than 60% by volume, the variation in conductivity (resistance) when the compound is under pressure, from the conductivity level when the compound is not under pressure, is insignificant, the compound being thus of no practical use. Therefore, the proportion of the particles should be withing the range of 20 vol % to 60 vol %.

In accordance with the invention, the spherical particles of a macromolecular material have conductivity imparted to them by being baked and thereby wholly or partially carbonized. This process facilitates the selection of particle size for the conductive particles. It is thus possible to use particles having a uniform particle size, and thereby obtain a compound having highly stable pressure-sensitive conductive properties. Furthermore, the compound is easy to manufacture.

The degree of carbonization of the particles (i.e. the thickness of the carbonized portion of each particle's spherical shell) can be varied by changing the degree of baking of the paricles, and thus particles of varying grades of conductivity can be easily produced. It is, therefore, possible to obtain differing pressure-sensitive conductive characteristics without changing the mechanical properties of the compound.

The invention will be described further, by way of example, with reference to the accompanying drawing, in which:
Figs. 1a to 1c, inclusive, are sectional illustrations showing various degrees of carbonization of spherical particles of a macromelecular material as incorporated in exemplified compounds in accordance with the invention. In Fig. 1a, only the surface area of the particle is carbonized. In Fig. 1b, almost the entire particle is carbonized. In Fig. 1c, the particle is entirely carbonized;
Fig. 2 is a graph showing the pressing force-resistance relationships in Example 1; and
Fig. 3 is a graph showing the pressing force-resistance relationships in Examples 2 and 3, in which graph the reference character (a) represents such relationships in Example 2 and the reference character (b) represents those in Example 3.

Figs. 1a, 16 and 1c are schematic views showing a few examples of spherical carbonized particles used for the purpose of the invention. Particles of various grades of conductivity are shown as they are formed from non-conductivity spherical particles of a macromolecular material. Experiments have revealed that the electric conductivity of the particles varies according to the heating and baking conditions. This is considered to be attributable to the following facts. If, as in Fig. 1a, only a region around the outer periphery of a particle 1 is carbonized to a thickness (t) in a spherical shell pattern, the conductivity of the particle 1 is low because the carbonized portion 2, i.e. the portion having electric conductivity, is of a small volume relative to the total volume (the non-carbonized portion being designated by reference numeral 3). If carbonization progresses further to the extent that a larger part of the particle 1 is carbonized, as shown in Fig. 1b, the conductivity of the particle 1 becomes considerably greater. Finally, if carbonization progresses still further until the particle is completely carbonized, the conductivity of the particle is maximised. Thus, even if particles 1 of the same diameter are used, the degree of carbonization of the particles varies according to the baking conditions applied. These facts are considered to be responsible for the variations in conductivity which can be obtained in different embodiments of the invention.

The degree of carbonization of the particles 1 is adjustable by changes in baking conditions, such as heating temperature and time. Therefore, by baking and carbonizing preselected particles 1 of the specified diameter under preset baking conditions it is possible to obtain quite easily, particles 1 having the required conductivity.

Particular examples are given hereinbelow to further illustrate the invention.

### Example 1

Spherical particles of a polystyrene resin material cross-linked with divinylbenzene and having a particle diameter of about 70 to 130 um were heated to 300°C in an air current, then heated and baked to 1000°C in an inert gas. The particle diameter measurements of the carbonized particles thus obtained showed that more than 90 wt% of the particles prior to baking were within the range of 53 to 105 pm. One hundred parts by weight of the carbonized particles within this diameter range were mixed with 100 parts by weight of a silicone rubber (TSE 270 - 4 U, produced by Toshiba Silicone Co.), the mixture being kneaded, and one form of the pressure-sensitive conductive elastomer compound according to the invention was thus produced.

The compound was moulded by press-moulding into a sheet having a thickness of 0.5 mm. Pressure was applied to the sheet by a rod-like pressing electrode having a 5 mm diameter, and the relationships between the pressing force and the resistance were measured. The measurements as shown in Fig. 2 revealed satisfactory resistance variation characteristis, with only a small degree of hysteresis.

In this example, the fine spherical particles of polystyrene resin were produced in the following way. Benzoyl peroxide or lauroyl peroxide was dissolved in a mixed monomer liquid of styrene a divinylbenzene, and the resulting liquid was vigorously agitated in water to which a dispersant, such as completely-saponified polyvinylalcohol, non-completely-saponified polyvinyl-alcohol or the like had been added, then suspension polymerized at 80°C for 6 to 8 hours.

### Example 2

A phenolic resin having a spheric particle configuration and a particle diameter of about 60 to 100 pm was heated and baked at 800°C in an inert gas. The particle diameters of the carbonized spherical particles thus obtained in glass-like (amorphous) form were such that more than 90 wt % of the particles prior to baking were within the range of 44 to 74 um. One hundred parts by weight of the carbonized particles within this range were mixed with 100 parts by weight of same silicone rubber as in Example 1, the mixture being kneaded together, then moulded by press moulding into a sheet having a thickness of 0.5 mm.

Pressing force-resistance characteristics were measured in same way as in Example 1. The measurements, as shown in Fig. 3 graph (a), revealed that the sheet had good characteristics, with a small degree of hysteresis.

In this example, the spherical phenolic resin particles were produced in the following way. A resol resin was dissolved in acetone, and a precipitant was added to the mixture during stirring, so that fine spherical resin particles were separated out. The particles were then subjected to filtration and drying and subsequently heated and hardened.

Spherical phenolic resin particles were also produced in the following way. Phenol was added to a large amount of an aqueous solution of hydrochloric acid and formaldehyde during stirring, whereby solid matter having a spherical configuration was produced. The solid matter was separated out, then neutralized in an alkaline solution, and subsequently washed in water and dried. Use of the phenolic resin particles thus obtained also gave satisfactory results as in aforesaid case.

### Example 3

Spherical phenolic resin particles identical with those used in Example 2 were heated and baked at 600°C. The particle diameters of the glass-like spherical carbonized particles were such that more than 90 wt % of the particles prior to baking were within the diameter range of 44 to 74 ¡lm. One hundred and twenty parts by weight of the carbonized particles within this range were mixed with 100 parts by weight of same silicone rubber as in Example 1, the mixture being kneaded together and a 0.5 mm thick sheet was produced by press-moulding.

Measurements were made in same way as in Example 1. The results are shown in Fig. 3 graph (b). In this instance, the variations in resistance shown are of a similar pattern to those in Example 2 except that the range of variations is different. This indicates that the conductivity of the spherical phenolic resin particles varies according to the baking temperature for the particles. Presumably, this is due to the face that the degree of carbonization varies according to the baking temperature and that as the baking temperature becomes higher, the carbonized portion of each particle will become greater. In other words, it is considered that the thickness (t) of the carbonized spherical shell portion in Fig. 1a becomes greater at a higher baking temperature and as the carbonized portion is increased so the conductivity of the particle is increased.

## Claims

1. A method of manufacturing a pressure-sensitive conductive elastomer compound comprising the steps of:
(a) forming spherical particles of macromolecular material of 30 to 120 pm in diameter by chemical pulverization or suspension polymerization;
(b) at least partially carbonizing said spherical particles by baking them within inert gas (without addition of carbon); and
(c) incorporating and dispersing the resultant carbonized spherical particles into a matrix material having insulating and elastomeric properties, the proportion of particles to the entire compound being 20 to 60 % by volume.

2. A method according to claim 2, wherein the spherical particles are formed of polystyrene resin by adding polymerization catalyst to styrene monomers and stirring this mixture in water along with addition of a dispersant such that the monomers disperse in oil-drop form and then polymerize.

3. A method according to claim 1, wherein the spherical particles are formed of phenol resin by dissolving resol resin into acetone and stirring this solution along with addition of percipitant so that said resin particles separate out.

4. A method according to any preceding claim wherein the spherical particles are carbonized by baking at a temperature in the range of 600°C to 1,000°C.

5. A method according to any preceding claim wherein the matrix material is silicone rubber.

## Patentansprüche

1. Verfahren zur Erzeugung eines druckempfindlichen leitfähigen Verbundelastomers mit folgenden Verfahrensschritten:
a) Bildung runder Teilchen aus makromolekularem Material von 30 bis 120 um Durchmesser durch chemische Pulverisation oder Suspensionspolymerisation;
b) mindestens teilweises Karbonisieren der runden Teilchen durch Backen in inertem Gas (ohne Zusatz von Kohlenstoff); und
c) Einschließen und Verteilen der sich ergebenden karbonisierten runden Teilchen in einem Matrix-Material, das isolierende und elastomerische Eigenschaften hat, wobei der Anteil der Teilchen an der gesamten Zusammensetzung 20 bis 60 Volumenprozent beträgt.

2. Verfahren nach Anspruch 1, dadurch gekennzeichent, daß die runden Teilchen aus Polystyrolharz unter Hinzufügen von Polymerisationskatalysatoren zu Styrolmonomeren und Rühren dieser Mischung in Wasser unter Hinzufügen eines Dispersionsmittels gebildet werden, dergestalt, daß die Monomere in Öltropfenform dispergieren und dann polymisieren.

3. Verfahren nach Anspruch 1, dadurch gekennzeichnet, daß die runden Teilchen aus Phenolharz durch Auflösen von Resolharz in Azeton und Rühren dieser Lösung unter Hinzufügen von Ausscheidungsmittel gebildet werden, dergestalt, daß die Harzteilchen ausfallen.

4. Verfahren nach einem der vorangehenden Ansprüche, dadurch gekennzeichnet, daß die runden Teilschen durch Backen bei einer Temperatur in dem Bereich von 600°C bis 1,000°C karbonisiert werden.

5. Verfahren nach einem der vorangehenden Ansprüche, dadurch gekennzeichnet, daß das Matrix-Material Silicongummi sit.

## Revendications

1. Procédé de fabrication d'un matériau composite conducteur sensible à la pression à base d'élastomère, dans lequel:
(a) on forme par pulvérisation chimique ou polymérisation en suspension, des particules sphériques de 30 à 120 um de diamètre, d'une metériau macromoléculaire;
(b) on carbonise au moins partiellement ces particules sphériques, en les cuisant dans un gaz inerte (sans ajouter de carbone); et
(c) on incorpore et on disperse les particles sphériques carbonisées résultantes, dans un matériau de matrice ayant des propriétés isolantes et d'élastomère, la proportion de particules dans l'ensemble de la composition étant de 20 à 60 % en volume.

2. Procédé selon la revendication 2, dans lequel les particules sphériques, sont formées à partir d'une résine de polystyrène, en ajoutant un catalyseur de polymérisation à des monomères dérivés de styrène, et en agitant ce mélange dans de l'eau tout en ajoutant un agent dispersant, de telle façon que les monomères soient dispersés sous la forme de gouttes d'huile et polymérisent ensuite.

3. Procédé selon la revendication 1, dans lequel les particules sphériques son formées à partir d'une résine phénolique, en dissolvant une résine de résol dans de l'acétone, et en agitant cette solution tout en ajoutant un agent précipitant, de façon à ce que les particules de résine soient séparatées.

4. Procédé selon l'une quelconque des revendications précédentes, dans lequel les particules sphériques sont carbonisées par cuisson à une température do 600°C à 1000°C.

5. Procédé selon l'une quelconque des revendications précédentes, dans lequel le matériau de matrice, est un caoutchouc de silicone.
